

## 1

3,573,245

## STABILIZED POLYAMIDES

Gerhard Mueller, Limburgerhof, Pfalz, and Helmut Doerfel and Hans Wilhelm, Ludwigshafen (Rhine), Germany, assignors to Badische Anilin- & Soda-Fabrik Aktiengesellschaft, Ludwigshafen (Rhine), Germany

No Drawing. Filed Aug. 29, 1967, Ser. No. 663,942

Int. Cl. C08g 51/56

U.S. Cl. 260—45.75

5 Claims

## ABSTRACT OF THE DISCLOSURE

Stabilization of polyamides by adding of iodine compounds and copper complexes of compounds containing twice to four times the structural unit:



in which X denotes a hydrocarbon radical having one or two carbon atoms.

It is known that polyamides can be stabilized against the effect of heat and air by adding compounds containing phenolic groups. The numerous phenolic compounds proposed for this purpose all have the disadvantage, however, that they discolor the polyamide upon prolonged action of heat in the presence of air. Discoloration of the polyamide often takes place even during the incorporation of these phenolic stabilizers.

Condensation products of aliphatic aldehydes with aromatic or cycloaliphatic amines have also already been recommended for stabilizing polyamides. These stabilizers however also cause discoloration of the polyamides.

Copper or compounds of copper, such as copper acetate, copper salts of phosphoric acid and hypophosphoric acid, alone or in combination with cerium (III) and/or titanium (III) salts, have also been suggested as heat stabilizers for polyamides. The effect of the copper compounds can be increased by using them in the form of copper complexes, either alone or together with halogen compounds, particularly iodine compounds. Examples of compounds proposed for forming complexes are phosphorus compounds and amines. These compounds however decompose during polycondensation, lower the degree of polycondensation of the polyamide or cannot be distributed homogeneously in the polyamide.

We have now found that polyamides can be stabilized against the effect of heat particularly effectively without the said disadvantages by using as the stabilizing agent an iodine compound together with a copper complex of a compound which contains twice to four times the structural element:



in which X denotes a hydrocarbon radical having one or two carbon atoms.

The following are examples of compounds which may be used according to this invention for preparing the copper complex: imidodiacetic acid, ethanolaminodiacetic acid, nitrilotriacetic acid, anilino-N,N-diacetic acid, cyclohexylenediamino - N,N' - tetraacetic acid, 2,6-diaminomethyl - 4 - methylphenol - N,N' - tetraacetic acid, N'-methyl diethylenetriamino - N,N' - tetraacetic acid and bis(β-aminoethyl)ether-N,N'-tetraacetic acid.

Tetraacetic acid derived from aliphatic and alicyclic 1,2-diamines, such as ethylenediamine-N,N'-tetraacetic acid and 1,2-diaminocyclohexane-N,N'-tetraacetic acid, and also the diacetic acid derived from β-aminoethanol, are particularly suitable.

## 2

Production of these acids and their complex copper salts form no part of the subject-matter of the present invention. The acids may be obtained for example by alkylation of ammonia or amines with α-halofatty acids or by condensation of carbonyl compounds with amines and hydrogen cyanide followed by hydrolysis of the nitrile group. The compounds may also be obtained by oxidation of ethanolamines.

The copper complexes used as stabilizers may be prepared by reaction of the acids with copper compounds, such as copper acetate or copper hydroxide. The copper complexes according to this invention contain in the molecule carboxyl groups which are not utilized in the formation of the complex; they therefore behave as polyamide-formers and may be wholly or partly condensed into the polyamides to be stabilized. In these cases the stabilizers adhere particularly strongly to the polymers and cannot be removed by extraction.

For the stabilization of the polyamides, 0.002 to 0.5%, preferably 0.01 to 0.25%, of the copper complex is used, the optimum amount of the stabilizer used depending on its constitution and on the polyamide. The copper complexes may be used in the form of free acids or in the form of their alkali metal or amine salts. They are used in combination with an iodine compound, such as an alkali metal iodide, ammonium iodide, an iodide of a diamine or an organic iodine compound such as an iodo-lactam, for stabilizing polyamides in accordance with the process of the invention. The iodine compounds may be used in an amount of one to hundred times the weight of the copper complex.

The mixture of copper complex and iodine compound to be used according to the process of the invention may be added to the polyamide-forming starting materials prior to the formation of the polyamide or may be incorporated into the polyamide. The effect of the new stabilizer systems extends to all polyamides and copolyamides from the known polyamide-forming compounds, such as lactams, diamines and dicarboxylic acids or aminocarboxylic acids.

It is a special advantage that the new stabilizers may be added to the polyamide starting materials because they do not separate any copper or copper oxide under the conditions of the polycondensation. They condense into the polyamide and are firmly bonded in the polymer so that in a subsequent extraction of the polycondensate for removal of monomers and oligomers, only very small amounts of stabilizer are removed. The new copper complexes are superior to other copper compounds in that they do not result in any discoloration of the polyamide formed during the polycondensation.

It is surprising that complexes in which the copper ions are so strongly masked as they are in those used in accordance with this invention should have so excellent a stabilizing effect for polyamides against the effect of heat. Owing to their stability, their effectiveness is maintained even under prolonged action of heat at relatively high temperatures.

Polyamides stabilized by the process according to this invention are suitable for the production of moldings, films, sheeting, bands, ribbons, tapes and fibers for a great variety of purposes.

The following examples further illustrate the invention; the parts specified in the examples are parts by weight.

65

## EXAMPLE 1

60 parts of the salt of adipic acid and hexamethylene diamine and 40 parts of epsilon-caprolactam are polycondensed for three hours at 270° C. with 20 parts of water, 0.017 part of the copper dipotassium salt of ethylenediaminetetraacetic acid and 0.15 part of potassium iodide. The K value of the copolymer is 69 and rises to

## 3

86 after it has been annealed for three days at 140° C. in air. The light absorption (measured in pressed plates 1 mm. in thickness) is 23% prior to annealing and 58% after three days. After this period, the polycondensate is not embrittled.

## EXAMPLE 2

60 parts of the salt of adipic acid and hexamethylene-diamine and 40 parts of epsilon-caprolactam are mixed with 20 parts of water, 0.068 part of the copper-dipotassium salt of ethylenediaminetetraacetic acid and 0.9 part of potassium iodide and polycondensed as in Example 1. The K value of the polyamide is 71. The K value is 90 after the material has been left for three days at 140° C. in air. The light absorption rises from 18% to 54% after the three-day heat treatment.

## EXAMPLE 3

60 parts of the salt of adipic acid and hexamethylene-diamine and 40 parts of epsilon-caprolactam are mixed with 20 parts of water, 0.028 part of the copper salt of ethylenediaminetetraacetic acid and 0.3 part of potassium iodide and then poly-condensed as in Example 1. The K value of the polycondensate is 73. After a heat treatment at 140° C. for three days, the K value has increased to 87. The light absorption prior to the heat treatment is 26; after three days it is 61%. The polyamide is not embrittled after this treatment.

## EXAMPLE 4

60 parts of the salt of adipic acid and hexamethylene-diamine and 40 parts of epsilon-caprolactam are homogeneously mixed with 20 parts of water, 0.055 part of the copper salt of ethylenediaminetetraacetic acid and 1.2 parts of potassium iodide and polycondensed as described in Example 1. A polycondensate is obtained having a K value of 67 which rises to 87 after annealing for three days at 140° C. in air. The light absorption is 15% and, after three days heat treatment, 53%.

## EXAMPLE 5

The procedure of Example 1 is followed but with the addition according to the invention of 0.074 part of the copper-hexamethylenediamine salt of ethylenediaminetetraacetic acid. A polyamide is obtained having a K value of 69. Testing the resistance to heat at 140° C. in air gives a K value of 91 after three days storage. The light absorption prior to the heat treatment is 22 and after the heat treatment 43%. The polycondensate is not embrittled after this period.

## EXAMPLE 6

100 parts of caprolactam is polycondensed for three hours at 270° C. with 20 parts of water, 0.074 part of the copper-hexamethylenediamine salt of ethylenediaminetetraacetic acid and 0.9 part of potassium iodide. The pressure is then released at 270° C. to remove excess steam and the product is condensed for three hours at 270° C. in a stream of nitrogen. The polycondensate is granulated, boiled up twice with water for twelve hours and dried. The K value of the polycondensate is 68 and rises to 83 after storage for three days at 140° C. and to 87 after ten days. The product is not embrittled after this period.

## EXAMPLE 7

100 parts of caprolactam is polycondensed with 20 parts of water, 0.08 part of the copper salt of nitrilotriacetic acid and 0.9 part of potassium iodide as described in Example 6. The product is extracted and dried. The granulate is extruded into rods 50 x 6 x 4 mm. and stored in the air at 140° C. for three, five, seven and fourteen days. The rods are then conditioned for eight hours at 30° C. and 80% relative humidity. The impact strength of the annealed rods is tested according to DIN 53,453. 75

## 4

The rods show no fracture after hot storage for fourteen days.

## EXAMPLE 8

5 100 parts of caprolactam is polycondensed with 20 parts of water, 0.065 part of the copper salt of 1,2-diaminocyclohexane-N,N'-tetraacetic acid and 0.9 part of potassium iodide as described in Example 6, extracted and dried. The product is extruded into rods 50 x 6 x 4 mm. 10 and annealed, conditioned and tested according to DIN 53,453 as in Example 7. After storage for fourteen days at 140° C., the polycaprolactam is still so tough that no fracture occurs.

15

## EXAMPLE 9

The procedure of Example 8 is followed, but only 0.006 part of the copper salt of 1,2-diaminocyclohexane-N,N'-tetraacetic acid and 0.09 part of potassium iodide are added. A polyamide is obtained which shows no fracture 20 after storage for fourteen days while heating and testing according to DIN 53,453.

## EXAMPLE 10

25 100 parts of caprolactam is polycondensed with 20 parts of water, 0.06 part of the copper salt of ethanolamine-N,N-diacetic acid and 0.9 part of potassium iodide as described in Example 6. The product is extracted and dried. The polyamide chips are extruded into rods 50 x 6 x 4 mm. and the rods kept for three to fourteen 30 days in the air at 140° C., conditioned as in Example 7 and tested according to DIN 53,453. There is again no fracture of the test specimens which have been annealed for fourteen days.

35

## EXAMPLE 11

The procedure of Example 10 is followed with an addition of 0.006 part of the copper salt of ethanolamine-N,N-diacetic acid and 0.09 part of potassium iodide. A 40 polyamide is obtained having the same heat resistance as described under Example 10.

## EXAMPLE 12

100 parts of polycaprolactam is mixed with 1.065 parts 45 of the copper salt of ethanolamine-N,N-diacetic acid and 0.3 part of potassium iodide in a high-speed mixer and the product processed in a commercial extruder. The polyamide granulate is dried and extruded into rods 50 x 6 x 4 mm. which are stored for three to fourteen 50 days in the air at 140° C. and then for eight hours at 30° C. and 80% relative humidity. Tests of the impact strength according to DIN 53,453 did not cause fracture.

We claim:

1. A composition of matter stabilized against heat and light comprising a synthetic linear polyamide having recurring



60 groups in the main chain of the molecule, there being incorporated in said polyamide a stabilizing mixture of:

(a) about 0.002 to 5% by weight, with reference to the polyamide, of a copper complex of an organic compound selected from the class consisting of monoamines bearing at least two  $-\text{CH}_2-\text{COOH}$  substituents on the nitrogen atom and diamines in which each terminal nitrogen atom bears two



substituents thereon; and

(b) about 0.002 to 2.5% by weight, with reference to the polyamide, of an iodide selected from the class consisting of alkali metal iodides, alkaline earth metal iodides and ammonium iodide.

2. A composition as claimed in claim 1 wherein component (b) is potassium iodide.
3. A composition as claimed in claim 1 wherein component (a) is a copper complex of ethylenediamine-N,N'-tetracetic acid.
4. A composition as claimed in claim 1 wherein component (a) is a copper complex of ethanolamine-N,N'-diacetic acid.
5. A composition as claimed in claim 1 wherein component (a) is a copper complex of 1,2-diaminocyclohexane-N,N'-tetraacetic acid,

## References Cited

## UNITED STATES PATENTS

|             |        |           |       |           |
|-------------|--------|-----------|-------|-----------|
| 2,705,227   | 3/1955 | Stamatoff | ----- | 260—45.7  |
| 3,294,735   | 9/1966 | Twilley   | ----- | 260—45.75 |
| 5 3,313,769 | 4/1967 | Maahs     | ----- | 260—45.75 |

DONALD E. CZAJA, Primary Examiner

V. P. HOKE, Assistant Examiner

10

U.S. Cl. X.R.  
260—45.7, 45.9, 78

UNITED STATES PATENT OFFICE  
CERTIFICATE OF CORRECTION

Patent No. 3,573,245 Dated March 30, 1971

Inventor(s) Gerhard Mueller et al

It is certified that error appears in the above-identified patent and that said Letters Patent are hereby corrected as shown below:

Column 1, line 7, insert -- Claims priority, application Germany, September 9, 1966, P 15 95 342.1 --.

Column 2, line 64, "specifield" should read -- specified --.

Column 3, line 25, "thre" should read -- three --; line 36, "scrbed" should read -- scribed --.

Signed and sealed this 14th day of September 1971.

(SEAL)

Attest:

EDWARD M. FLETCHER, JR.  
Attesting Officer

ROBERT GOTTSCHALK  
Acting Commissioner of Pat